

Nov. 24, 1970

R. L. SIMONTON

3,541,831

EXTRUSION MANDREL

Filed April 7, 1967

2 Sheets-Sheet 1

Ti q. 1.



Ti q. 2.



Ti q. 3.



Ti q. 4.



Ti q. 5.



Ti q. 4A.



INVENTOR.

RAYMOND L. SIMONTON

BY

M. L. Pinel

ATTORNEY

Nov. 24, 1970

R. L. SIMONTON

3,541,831

EXTRUSION MANDREL

Filed April 7, 1967

2 Sheets-Sheet 2



INVENTOR.

RAYMOND L. SIMONTON

BY

*M. L. Pineel*

ATTORNEY

3,541,831  
**EXTRUSION MANDREL**  
Raymond L. Simonton, Huntington, W. Va., assignor to  
The International Nickel Company, Inc., New York,  
N.Y., a corporation of Delaware  
Filed Apr. 7, 1967, Ser. No. 629,162  
Int. Cl. B21c 25/06  
U.S. Cl. 72—266

15 Claims

## ABSTRACT OF THE DISCLOSURE

Compound mandrel for use in hot extrusion of hollow metal products has a heat-resistant casing disposed around a tension bar of maraging steel.

The present invention relates to metal working apparatus and, more particularly, to apparatus for extruding hollow metal articles.

Heretofore, in the metallurgical art, methods and apparatus have been developed for forming hollow metal articles such as seamless tubes by extruding a heated metal billet over a mandrel and through a die. For instance, hot extrusion of tubular products made of high strength, difficultly formable, high melting point metals such as carbon steel, stainless steel and other difficult to form metals is described in "The Making, Shaping and Treating of Steel," 8th edition, U.S. Steel, 1964.

During hot extrusion of tubular products, the mandrel is subjected to severe heat and to a complex combination of forces including transverse compressive forces from the billet which is being compressed within the extrusion chamber, longitudinal tensile forces that are exerted through friction of the extruded metal passing over the mandrel and also transverse bending forces. Although theoretical considerations might indicate that the forces on a mandrel would be exerted symmetrically with respect to the longitudinal axis of the mandrel, it has been found in practice that mandrels, especially mandrels of relatively small cross section, are sometimes bent or broken in bending by the complex forces of extrusion. Additionally, thermal shock from contact with hot billets and from cooling between extrusions exerts severe stresses in hot extrusion mandrels and sometimes results in unsatisfactory short life of hot extrusion mandrels, particularly where the mass of the mandrel is high such as in mandrels of 5-inch diameter or larger. Materials without good thermal shock resistance are not wholly satisfactory for hot extrusion mandrels even if characterized by high strength and other desirable properties. For instance, breakage due to thermal shock has resulted in unsatisfactorily short life of mandrels made of tool steel having a nominal composition of 0.35% carbon, 5% chromium, 1% vanadium and 1.5% molybdenum. The poor thermal shock properties which generally characterize cemented carbide materials would be expected to render these materials unsatisfactory for hot extrusion mandrels. Extrusion mandrels are also subjected at times to heavy mechanical shocks which cause breakage if the toughness of the mandrel is inadequate. Further difficulties with mandrels in the prior art, e.g., 5% chromium tool steel mandrels, include heat checking, cracking, wear, scoring and tearing of the exterior surfaces.

In view of the stresses and strains and the heat to which extrusion mandrels are subjected, it is not surprising to find that the mandrels fail undesirably frequently. The effects of the complex forces and the heat, shock, friction, etc., to which hot extrusion mandrels are subjected are so various and interrelated as to make it im-

practical to precisely predict all the requisite characteristics for satisfactory extrusion mandrel structures and materials. Accordingly, the art of extrusion mandrel design is largely empirical. Due to the high cost of metal and machining for replacing extrusion mandrels, the failure thereof contributes disadvantageously to increasing the cost of producing extruded hollow metal articles. Additionally, mandrel failure results in costly spoilage of extrusion billet material and loss of production time. For instance, when the head portion is pulled from a mandrel during extruding a tube, usually the head becomes lodged in the tube and the remainder of the billet is extruded as a solid bar instead of as the desired tube. Scoring and other surface deterioration of the mandrel detrimentally results in interior surface defects in the extruded products, due to lack of a smooth surface on the mandrel.

In attempting to overcome mandrel failure problems, the art has provided internal water-cooling means in 20 mandrels with the object of maintaining the strength of the metal when surrounded by a heated billet. However, water-cooled mandrels in the prior art suffer from further disadvantages and have not overcome all problems of mandrel failure, one disadvantage being that water-cooling passages decrease the amount of metal available 25 for strength. A further disadvantage of water cooling is that in event of rupture of the mandrel, water can flow into the interior of the hot billet and the resulting steam pressure confined in the extrusion chamber can 30 do great damage, such as by violently exploding the partially extruded tube from the press. Accordingly, a high margin of strength is needed for safety in water-cooled hot-extrusion mandrels. Other attempts to provide improved mandrels for hot extrusion include application of 35 hard facing coatings, e.g., tungsten-carbide coatings, high-carbon cobalt alloy coatings and high-carbon steel coatings, but hard facing coatings have suffered from cracking difficulties.

Although many attempts were made to overcome the 40 foregoing difficulties and other difficulties, none, as far as I am aware, was entirely successful when carried into practice commercially on an industrial scale.

It has now been discovered that a new structure having 45 a new combination of characteristics provides an extrusion mandrel having improved resistance to fracture or rupture and improved wear resistance, whereby increased service life is obtained.

It is an object of the present invention to provide a new extrusion mandrel having improved resistance to 50 failure by deformation or fracture, including resistance to tensile failure, and also having improved resistance to wear, tear and scoring of the outer surface.

A further object of the invention is to provide a new 55 mandrel for use in extruding hollow articles made of metals characterized by high resistance to deformation, heat resistance and/or high melting points.

Other objects and advantages will become apparent from the following description taken in conjunction with the accompanying drawings in which:

60 FIGS. 1, 2, 3 and 4 illustrate, in longitudinal cross section, four embodiments of the mandrel provided in accordance with the invention; and

FIG. 4a illustrates a transverse cross section of the 65 mandrel of FIG. 4.

FIG. 5 shows a side view of the mandrel of FIG. 4 attached to a mandrel holder of an extrusion press with the mandrel holder shown in longitudinal partial cross section.

70 FIG. 6 illustrates, in partial cross section, cooperation of an extrusion die and metal being extruded into tubular form with the mandrel of FIG. 4.

Generally speaking, the present invention is directed to a new extrusion mandrel comprising a high strength, ductile, tension bar composed of maraging steel having a heat treated, aged, internal structure characterized by a yield strength of at least about 200,000 pounds per square inch (p.s.i.) and a tensile elongation of at least 7%, advantageously at least about 10%, at room temperature, a full length casing composed of a ductile heat resistant alloy slidably disposed around the tension bar and a retainer at the forward end of the tension bar. The retainer is engageable with the front end, i.e., the forward portion near or at the forward extremity, of the casing and is adapted to limit forward motion of the casing, thereby restraining the casing from being dragged off the tension bar during extrusion. At the rearward end of the tension bar a threaded stud or other attachment means is provided for mounting the mandrel in an extrusion press. It is to be particularly noted that the mandrel components are so arranged that forward longitudinal movement of the casing is mechanically restrained only by the retainer and only at the front end of the casing. The ductile heat resistant casing is characterized by ductility that avoids fracture in event of moderate bending such as can occur during extrusion, by metallurgical stability and also by good retention of hardness and strength when heated to elevated temperatures. Additional characteristics of the casing include thermal shock resistance and wear and abrasion resistance at high temperatures.

During use, when a billet is being extruded over the mandrel, the tension bar sustains essentially all the tensile load exerted by friction of the forward moving billet metal and, inasmuch as the casing is slidably disposed on the tension bar and is restrained by the retainer only at the front end of the casing, the casing is under longitudinal compression and is not subjected to tensile loading. It is to be understood herein that reference to compression in a mandrel component refers to compression in the component when taken as a whole. Thus, where the casing as a whole is in compression it is referred to as being in compression and not in tension even though small portions of the casing may be subjected to some highly localized tensile stress, for instance, tensile stress such as may be exerted on the outer skin of the casing by friction where forward-moving extrusion metal contacts the casing. Of course, during extrusion the casing is also subjected to complex stresses including transverse compression in addition to longitudinal compression. Transverse compressive forces on the casing are transmitted to the tension bar, which resists transverse compression of the casing and thereby serves as a back-up for the casing. Thus, the tension bar is sometimes simultaneously in transverse compression and longitudinal tension. It is further pointed out that the full length casing extends over essentially the entire length of the tension bar, thereby preventing wear, scoring and other surface damage to the tension bar and also protecting the tension bar against heat.

Maraging steels referred to herein are iron-base alloys, i.e., alloys wherein the percentage of iron is greater than the percentage of any other element present in the alloy, and are generally characterized by low carbon contents not greater than about 0.15% carbon, advantageously not greater than 0.05% carbon, more advantageously not greater than 0.03% carbon. In addition to iron, maraging steels generally contain about 10% to about 30% nickel, up to about 30% cobalt, up to about 10% molybdenum and up to about 8% chromium and also contain auxiliary hardening elements such as titanium, aluminum and/or columbium. Such steels are described in U.S. Pats. Nos. 3,093,518 and 3,093,519. In commercial practice, tensile strength levels, e.g., 250,000 p.s.i. yield strength, are commonly employed in designating maraging steels. Yield strengths referred to herein are determined by the 0.2% offset method; tensile elongations are with one-inch gage lengths. Advantages of the new mandrel tension bar hav-

ing, in accordance with the invention, a maraged micro-structure include high tensile strength, ductility, toughness and freedom from detrimental deformation during heat treatment. Ductility and toughness, including high notch tensile strength, are especially required for mandrels wherein the tension-supporting member is of low cross-sectional area, such as in fluid cooled mandrels and in mandrels of small diameter, e.g., 2 $\frac{1}{2}$  inches or less diameter, in order to avoid cracking or fracture due to bending.

In carrying the invention into practice, it is highly advantageous, in order to provide a mandrel having especially high resistance to tensile failure, that the mandrel comprise a maraging steel tension bar characterized in the heat treated (maraged) condition by high yield strength of at least about 250,000 p.s.i. at room temperature. Advantageous high strength embodiments of the tension bar include tension bars made of maraging steel containing about 17% to about 19% nickel, about 7% to about 9.5% cobalt, about 3% to about 5.2 molybdenum, about 0.15% to about 0.8% titanium, about 0.05% to about 0.15% aluminum, up to about 0.03% carbon with the balance essentially iron and heat treated to have a yield strength on the order of about 250,000 p.s.i. or higher and a tensile elongation of at least about 10%, e.g., 12%, at room temperature, e.g., heat treated by heating for about 1 hour at about 1500° F. followed by air cooling and reheating for about 3 hours at about 900° F. and then air cooling. Toughness is needed in the tension bar and use therein of brittle materials, or materials which are susceptible to embrittlement upon exposure to temperatures encountered by mandrels during extrusion, is avoided. In order to obtain full benefits of the maraging steel tension bar in accordance with the invention it is advantageous, especially in mandrels for hot extrusion of alloys such as nickel-base alloys, iron-base alloys or cobalt-base alloys, that such mandrels also have fluid coolant means for maintaining the temperature of the tension bar at less than 900° F., e.g., 700° F. or lower, thereby maintaining in use the high yield strength of the bar.

The ductile heat resistant alloy casing provided by the invention is composed of a metallurgically stable alloy containing at least 50% nickel, cobalt and/or iron, e.g., a metallurgically stable alloy containing up to about 21% chromium, advantageously 12% to 21% chromium, up to about 3.5% aluminum, up to about 3% titanium, up to about 6% columbium and/or tantalum, up to about 10% molybdenum, up to about 1% silicon, up to about 2% manganese, up to about 0.2% carbon and balance essentially metal from the group consisting of nickel, cobalt and iron. Advantageously, the casing is characterized at temperatures from room temperature up to at least about 1000° F. by ductility equal to at least 10% tensile elongation and by ultimate tensile strength of at least about 120,000 p.s.i. The casing of the new mandrel is metallurgically stable in the sense that the alloy matrix of the casing does not readily undergo any major phase change when subjected to heating and cooling under hot extrusion conditions. For instance, where the casing is an iron-base alloy the casing matrix is normally austenitic at room and elevated temperatures; casings made of alloys which undergo transformations from austenite to martensite, or vice versa, when heated and/or cooled under hot extrusion conditions are not in accordance with the present invention. Advantageous heat resistant alloys for the casing include ductile nickel-chromium alloys containing about 12% to about 21% chromium, up to about 28% iron, up to about 34% cobalt, up to about 3.5% aluminum, up to about 3% titanium, up to about 6% columbium or columbium plus tantalum, up to about 10% molybdenum, up to about 1% silicon, up to about 2% manganese and up to about 0.2% carbon with balance substantially nickel in an amount not less than about 45% of the alloy. All alloy composi-

tional percentages set forth herein are by weight. Alloys having precipitate-hardened microstructures, such as nickel-chromium alloys hardened with aluminum, titanium, columbium and/or tantalum, e.g., alloys containing 3%, or 3% to 7.5% or more of these elements, with good retention of hardness at elevated temperatures, are especially advantageous for the casing. Chemical compositions of some illustrative precipitation hardenable alloys for the ductile heat resistant casing of the new mandrel are set forth in the following Table I.

TABLE I

| Alloy No. | Percent |       |       |       |       |                 |       |      |                   |
|-----------|---------|-------|-------|-------|-------|-----------------|-------|------|-------------------|
|           | Cr      | Fe    | Co    | Al    | Ti    | Cb <sup>1</sup> | Mo    | C    | Ni                |
| 1-----    | 18      | 18.5  | ----- | 0.4   | 0.9   | 5               | 3     | 0.04 | Bal. <sup>2</sup> |
| 2-----    | 15      | 6.5   | ----- | 0.6   | 2.4   | -----           | ----- | 0.04 | Bal. <sup>2</sup> |
| 3-----    | 15      | 6.75  | ----- | 0.8   | 2.5   | 0.85            | ----- | 0.04 | Bal. <sup>2</sup> |
| 4-----    | 22      | 3     | ----- | ----- | ----- | 4               | 9     | 0.05 | Bal. <sup>2</sup> |
| 5-----    | 19      | ----- | 11    | 1.5   | 3     | -----           | 10    | 0.09 | Bal. <sup>2</sup> |

<sup>1</sup> Up to about 20% of the percentages shown for columbium may be tantalum.

<sup>2</sup> Bal. = Balance, which can include small amounts of deoxidizers, malleabilizers and nondetrimental impurities.

The slideable relationship of the casing to the tension bar is a sufficiently close fit, e.g., 0.005-inch clearance, to enable the bar to back-up the casing during extrusion and yet permit the casing to move freely enough to avoid being stressed longitudinally in tension by frictional forces during extrusion or by thermal expansion forces which may arise from differences in temperature or in thermal expansion coefficients of the casing and the tension bar. Close slideable fits which permit the casing to be moved on to the bar by hand or by an arbor press are satisfactory. Even though the casing can be press fit to the tension bar and during use may become even more tightly fit (but not welded) by extrusion, such fits are still slideable in relationship to the very high forces existent during extrusion or during heating and cooling of the mandrel before and after extrusion. In addition, the unbonded fit promotes flexural advantages for avoiding fracture in bending and permits removal of the casing for replacement when overly worn or when use of another size casing is required. In contradistinction to the slideable disposition of the casing on the tension bar in the mandrel of the invention, mandrels having coatings, casings, collars, etc., which are joined by bonding, e.g., welded, brazed, diffusion bonded, etc., and/or which are otherwise rigidly joined to a core, whether continuously joined or joined at front and rear portions of the casing, do not have all of the advantages of, and are not in accordance with, the present invention.

The retainer can be integral with the tension bar or can be replaceably fastened to the front end of the bar, e.g., held by a threaded stud at the front end of the bar. Where the retainer is not integral with the bar, the retainer and the fastening means therefor are advantageously made of high strength maraging steel inasmuch as the retainer is subjected to high forces tending to pull the retainer forwardly from the bar during extrusion.

A new mandrel which, in accordance with the invention, is particularly advantageous for hot extrusion of heat resistant nickel-chromium alloys comprises a casing made of a precipitate-hardened alloy containing about 50% to about 55% nickel, about 15% to about 21% chromium, 2% to 4% molybdenum, 4.75% to about 5.5% columbium, 0.65% to about 1.15% titanium, 0.2% to about 0.8% aluminum, up to about 0.1% carbon, advantageously 0.03% to 0.1% carbon, up to about 0.5% silicon, up to about 0.5% manganese with balance substantially iron, a tension bar composed of nickel-cobalt-molybdenum maraging steel in the condition characterized at room temperature by yield strength of at least about 250,000 p.s.i. and tensile elongation of at least about 10% and also comprising fluid coolant means for cooling the tension bar.

Turning now to the drawing, it is to be noted that

four specific embodiments of the new mandrel of the invention are illustrated therein. Each of the four illustrated mandrels is of uniform, circular, transverse cross section at the exterior surface and thus is adapted for extruding hollow cylindrical tubes having substantially uniform, circular, cross-sectioned interior passages. The components of the mandrels illustrated in FIGS. 1, 2 and 3 are all circular in transverse cross section.

FIG. 1 shows mandrel 10 having casing 11 slidably disposed around elongated, longitudinally extending tension bar 12 and abutting against retainer 13. Casing 11 extends essentially the entire length of tension bar 12. Threaded stud 14 is integral with bar 12 and is mated with threads 15 in the retainer. Extending from the rear end of the tension bar, threaded stud 16, which is integral with the bar, is adapted for attaching the mandrel to a mandrel holder in an extrusion press. (It is to be noted that, as referred to herein, a casing extends over essentially the entire length of a tension bar when the casing extends up to about the ends of the bar even though it does not extend over a stud or other connection means on the end of the bar.)

In FIG. 2, mandrel 20 comprises casing 21 and tension bar 22. Retainer 23 is integral with the tension bar. Casing 21 is slidably disposed over essentially the entire length of the tension bar and abuts against retaining shoulder 24 of retainer 23 at the forward end of the bar. Threaded stud 25 is integral with the rear of the bar and is adapted for attachment to a mandrel holder.

Mandrel 30, illustrated in FIG. 3, has casing 31 slidably disposed over the length of tension bar 32 and abutting against retainer 33. Mandrel 30 is adapted for piercing in addition to extruding and has detachable piercing point 34 fitted on stub 35. Threaded stud 36 provides means for attaching the mandrel to an extrusion press.

In FIG. 4, mandrel 40 has casing 41 slidably disposed over the entire length of grooved tension bar 42 and abutting against retainer 43. The retainer is mechanically fastened to the forward end of the bar by threaded stud 44 which is integral with the tension bar. The bar has central coolant passage 45 with inlet coolant pipe 46 extending into the central passage. Back flow of coolant in the passage is prevented by coolant seal 47. Transverse coolant ports 48 near the forward end of the bar enable coolant to flow from the central passage to coolant return grooves 49 and thence to transverse exit port 50. Grooves 49 are open to the casing, e.g., as illustrated in FIG. 4a, and thus provide for direct contact of the coolant with the casing. Coolant passing through port 50 can then flow rearward through the central passage and along the outside of the inlet pipe so as to exit at the rear of the mandrel.

FIG. 4a shows the transverse cross section of mandrel 40 taken at line 4a—4a of FIG. 4.

Mandrel 40 is shown, in FIG. 5, attached to mandrel holder 51 of an extrusion press. Threaded mounting stud 52, which is integral with the tension bar of the mandrel, is mated in thread 53 in the mandrel holder. Coolant passage 54 in the mandrel holder communicates with the central passage in the tension bar and coolant inlet pipe 46 extends rearward through passage 54 in the mandrel holder. Both the coolant inlet pipe and passage 54 communicate with coolant supply and coolant exhaust means, respectively, which are not shown and form no part of the invention.

FIG. 6 illustrates mandrel 40 and extrusion die 61 in extrusion press chamber 62 during extrusion of metal 63. It is understood that during normal operation the extrusion die is stationary and the mandrel moves with the mandrel holder of the extrusion press while the metal is extruded forwardly (to the right in FIG. 6) over the mandrel and through the die.

In the foregoing figures, it is to be noted that each of the mandrels is so arranged that the bar is a tension-sustaining member which, during extrusion, sustains es-

sentially all of the tensile force resulting from friction of the extrusion metal moving forwardly over the casing. Also, in each of the illustrated mandrels the casing is a compression-sustaining member which is placed in compression and is not loaded in tension when metal is being extruded over the mandrel.

For the purpose of giving those skilled in the art a better understanding of the invention and a better appreciation of the advantages of the invention, the following illustrative example is given:

An extrusion billet of a difficultly formable nickel-chromium-iron alloy having a nominal composition of about 15.8% chromium, 7.2% iron, 0.04% carbon, 0.2% manganese, 0.2% silicon and balance nickel and of a cylindrical configuration about 11 inches diameter and about 25 inches high, with an axially oriented hole about  $4\frac{1}{4}$  inches diameter drilled therethrough, was heated to a temperature of about  $2250^{\circ}$  F. and placed in the extrusion chamber of a forward extrusion press. An internally water-cooled mandrel in accordance with the invention was attached to the mandrel holder of the extrusion press. The mandrel casing was of hollow cylindrical configuration about 4 inches outside diameter, about  $2\frac{3}{4}$  inches inside diameter and about 36 inches length and was made of an alloy containing about 52.3% nickel, 18.6% chromium, 5.2% columbium-plus-tantalum, 3.1% molybdenum, 0.9% titanium, 0.5% aluminum, 0.3% silicon, 0.2% manganese, 0.04% carbon and balance essentially iron. The tension bar of the mandrel was made of maraging steel having a composition containing about 18% nickel, 9% cobalt, 5% molybdenum, 0.5% titanium, 0.1% aluminum and 0.01% carbon and in the heat treated condition characterized by a room temperature yield strength of about 300,000 p.s.i. The mandrel was inserted into the hole in the billet. Extrusion pressure was then exerted by the press and forced the billet metal over the mandrel and forwardly out through an extrusion die having a circular orifice about  $4\frac{1}{2}$  inches in diameter. The billet, which weighed about 500 to 600 pounds, was extruded in about 16 seconds to form an extruded tube over 40 feet long with an internal diameter of about 4 inches. When cooled, the tube was found to be of completely satisfactory quality without detrimental defects. The mandrel was further employed to make additional extruded tubes and was still in good useable condition after being used for at least about 200 extrusions. Normal life of conventional mandrels in such use is satisfactory for only about 40 or less extrusions.

Further illustration of the invention is afforded by the exemplary dimensions set forth in Table II, which shows mandrel diameters, tension bar diameters and casing wall-thicknesses (apart from clearances) for advantageous embodiments of the invention. The ratio of the casing wall thickness to the mandrel diameter is advantageously about 1:5 to about 1:9 for obtaining good results of long life without fracture in hot extruding heat resistant nickel-chromium alloys into tube forms having internal diameters from about 2 inches to about 9 inches.

TABLE II

| Mandrel diameter, inches | Tension bar diameter, inches | Casing wall thickness, inch |
|--------------------------|------------------------------|-----------------------------|
| 9                        | 7                            | 1                           |
| 7                        | 5                            | 1                           |
| 4                        | $2\frac{3}{4}$               | $\frac{5}{8}$               |
| $2\frac{1}{4}$           | $1\frac{1}{2}$               | $\frac{3}{8}$               |

It is to be observed that in the mandrel of the invention, having the casing in slidable relationship to the tension bar and having the casing extend the full length of the tension bar, except for a small longitudinal clearance gap, provides further advantages including extended useful life and increased scope of utility for the mandrel tension bar and other mandrel components apart from the casing. Thus, when the casing becomes worn beyond further usefulness or damaged, the casing can be re-

placed, thereby enabling continued use of the tension bar and other components. Further, for obtaining advantages of greater scope of utility, the new mandrel is provided with interchangeable casings of different external diameters and thus can be used for extruding a variety of different internal diameters in tubes. Such advantages of extended life and greater variety of use and also other advantages, including protection of the tension bar from heat and wear, could not be fully realized if the casing did not extend over essentially the entire length of the tension bar, e.g., at least about 90% of the working length, i.e., working surface, of the bar. Accordingly, the present invention is not to be confused with mandrels having relatively short lengths of special materials at portions of the mandrel exterior.

The present invention is particularly applicable in the hot extrusion of hollow metal articles made of alloys containing a major proportion, e.g., 50% or more, of nickel, iron and/or cobalt. The invention is also applicable in extrusion processes generally and is useful for cold extrusion where a mandrel having a replaceable wear-resistant outer casing and a tough, high strength, tension-sustaining interior is needed.

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and appended claims.

I claim:

1. An extrusion mandrel, for use with an extrusion press, comprising an elongated tension bar composed of maraging steel and characterized at room temperature by a yield strength of at least about 200,000 pounds per square inch and ductility equivalent to tensile elongation of at least 7%, an internal fluid coolant passage for transmitting fluid coolant to the tension bar, a ductile casing slidably disposed in unbonded contact on said tension bar and extending over essentially the entire length of the tension bar, a retainer at the forward end of the tension bar and adapted to limit forward movement of the casing and means for mounting the mandrel on an extrusion press.

2. An extrusion mandrel as set forth in claim 1 having a plurality of internal fluid coolant passages communicating with the casing.

3. An extrusion mandrel, for use with an extrusion press, comprising an elongated tension bar composed of maraging steel and characterized at room temperature by a yield strength of at least about 200,000 pounds per square inch and ductility equivalent to tensile elongation of at least 7%, a ductile casing slidably disposed in unbonded contact on said tension bar and extending over essentially the entire length of the tension bar, said casing being of a hollow cylindrical configuration with the ratio of the cylinder wall thickness of the casing to the mandrel diameter being about 1:5 to about 1:9, a retainer at the forward end of the tension bar and adapted to limit forward movement of the casing and means for mounting the mandrel on an extrusion press.

4. An extrusion mandrel, for use with an extrusion press, comprising an elongated tension bar composed of maraging steel and characterized at room temperature by a yield strength of at least about 200,000 pounds per square inch and ductility equivalent to tensile elongation of at least 7%, a ductile casing slidably disposed in unbonded contact on said tension bar and extending over essentially the entire length of the tension bar, said casing being composed of a ductile, metallurgically stable, heat resistant alloy containing at least about 50% of metal from the group consisting of nickel, cobalt and iron and characterized at temperatures from room temperature up to about  $1000^{\circ}$  F. by ductility at least equal to about

10% tensile elongation and by ultimate tensile strength of at least about 120,000 pounds per square inch, a retainer at the forward end of the tension bar and adapted to limit forward movement of the casing and means for mounting the mandrel on an extrusion press.

5. An extrusion mandrel as set forth in claim 4 wherein the maraging steel tension bar is characterized by a yield strength of at least about 250,000 pounds per square inch and ductility equal to at least about 10% tensile elongation at room temperature.

6. An extrusion mandrel as set forth in claim 5 wherein the casing is composed of a precipitate-strengthened alloy containing about 50% to about 55% nickel, about 15% to about 21% chromium, 2% to 4% molybdenum, 4.75% to about 5.5% columbium, 0.65% to about 1.15% titanium, 0.2% to about 0.8% aluminum, up to about 0.1% carbon, up to about 0.5% silicon, up to about 0.5% manganese with the balance essentially iron.

7. An extrusion mandrel as set forth in claim 6 having an internal coolant passage for transmitting fluid coolant to the tension bar.

8. An extrusion mandrel, for use in forward extrusion of a metal workpiece to form a hollow metal product, comprising

an elongated casing having a longitudinally extending exterior surface forming essentially the entire portion of the mandrel surface that contacts the workpiece during extrusion and also having a passage extending longitudinally through the full length of the casing;

an elongated tension bar closely fitted in unbonded contact with an interior wall of said passage in the casing and extending longitudinally the full length of the casing;

said tension bar being composed of maraging steel and having a maraged microstructure characterized at room temperature by a yield strength of at least about 200,000 pounds per square inch and ductility equivalent to tensile elongation of at least 7%;

retaining means secured to the tension bar and limiting forward movement of the front end of the casing; and

mounting means for securing the rearward end of the tension bar to an extrusion press;

said casing, tension bar, retaining means and mounting means being so disposed that during forward extrusion of a work piece over the mandrel the tension bar sustains essentially all the tensile load exerted on the mandrel by friction of the forward moving workpiece and the casing is under longitudinal compression.

9. An extrusion mandrel as set forth in claim 8 having an internal fluid coolant passage for transmitting fluid coolant to the tension bar.

10. An extrusion mandrel as set forth in claim 8 wherein the tension bar has a maraged steel microstructure characterized by at least about 10% tensile elongation at room temperature.

11. An extrusion mandrel as set forth in claim 8 wherein the tension bar has a maraged steel microstructure characterized by a yield strength of at least about 250,000 pounds per square inch at room temperature.

5. An extrusion mandrel as set forth in claim 8 wherein the casing is composed of a ductile, metallurgically stable, heat resistant alloy consisting essentially of about 12% to about 21% chromium, up to about 28% iron, up to about 34% cobalt, up to about 3% titanium, up to about 6% of metal from the group consisting of columbium and tantalum, up to about 10% molybdenum, up to about 1% silicon, up to about 2% manganese, up to about 0.2% carbon with the balance essentially nickel in an amount not less than 45% of the alloy and is characterized at temperatures from room temperature up to about 1000° F. by ductility at least equal to about 10% tensile elongation and by ultimate tensile strength of at least about 120,000 pounds per square inch.

13. An extrusion mandrel as set forth in claim 8 wherein the tension bar has a maraged steel microstructure characterized at room temperature by a yield strength of at least about 250,000 pounds per square inch and a tensile elongation of at least about 10% and wherein the casing has a precipitate-hardened microstructure characterized at temperatures from room temperature up to about 1000° F. by an ultimate tensile strength of at least about 120,000 pounds per square inch and a tensile elongation of at least about 10%.

14. An extrusion mandrel as set forth in claim 13 wherein the casing is composed of an alloy consisting essentially of about 50% to about 55% nickel, about 15% to about 21% chromium, 2% to 4% molybdenum, 4.75% to about 5.5% columbium, 0.65% to about 1.15% titanium, 0.2% to about 0.8% aluminum, up to about 0.1% carbon, up to about 0.5% silicon, up to about 0.5% manganese with the balance essentially iron.

15. An extrusion mandrel as set forth in claim 14 having an internal fluid coolant passage for transmitting fluid coolant to the tension bar.

#### References Cited

##### UNITED STATES PATENTS

|           |         |                     |        |
|-----------|---------|---------------------|--------|
| 2,184,048 | 12/1939 | Krause -----        | 72—273 |
| 2,809,750 | 10/1957 | Arenz -----         | 72—264 |
| 1,989,948 | 2/1935  | Singer -----        | 72—264 |
| 3,093,519 | 6/1963  | Decker et al. ----- | 148—31 |
| 3,093,518 | 6/1963  | Bieber -----        | 148—31 |

##### FOREIGN PATENTS

|           |        |                |
|-----------|--------|----------------|
| 1,445,277 | 8/1965 | France.        |
| 1,043,355 | 1/1964 | Great Britain. |

CHARLES W. LANHAM, Primary Examiner

55 A. L. HAVIS, Assistant Examiner

U.S. Cl. X.R.

72—253, 273